# EUROPEAN PATENT SPECIFICATION

(11) **EP 4 116 457 B1**
(45) Date of publication and mention of the grant of the patent: **08.05.2024**
(21) Application number: 20923408.7
(22) Date of filing: 29.10.2020
(51) Int. Cl.: C23C 2/06, B21D 22/20, C21D 1/18, C21D 9/00, C22C 18/04, C23C 2/28, C22C 38/00, C22C 38/60, C21D 9/48, C23C 2/40, C23C 28/00, C21D 1/673, C21D 7/13, C21D 8/02, C21D 9/46

(54) **HOT PRESSED MEMBER AND METHOD OF PRODUCING SAME. AND COATED STEEL SHEET FOR HOT PRESS FORMING**
HEISSGEPRESSTES BAUTEIL UND VERFAHREN ZU SEINER HERSTELLUNG, UND BESCHICHTETES STAHLBLECH FÜR HEISSPRESSEN
ÉLÉMENT PRESSÉ À CHAUD ET PROCÉDÉ POUR SA FABRICATION, ET TÔLE D'ACIER REVÊTUE POUR UN PRESSAGE À CHAUD

(30) Priority: 03.03.2020 JP 2020036054
(43) Date of publication of application: 11.01.2023
(73) Proprietor: JFE Steel Corporation, Tokyo 100-0011 (JP)
(72) Inventor: SATO, Rinta, Tokyo 100-0011 (JP); TANAKA, Minoru, Tokyo 100-0011 (JP); MIZUNO, Daisuke, Tokyo 100-0011 (JP); ANDO, Satoru, Tokyo 100-0011 (JP)
(74) Representative: Haseltine Lake Kempner LLP
(86) International application number: PCT/JP2020/040696
(87) International publication number: WO 2021/176768

(56) References cited:
- EP-A1- 3 009 526
- WO-A1-2014/122900
- WO-A1-2014/122900
- JP-A- 2001 348 678
- JP-A- 2005 113 233
- JP-A- 2005 113 233
- JP-A- 2012 112 010
- JP-A- 2012 112 010
- JP-A- 2013 241 671
- JP-A- 2013 241 671
- JP-A- 2019 531 413
- JP-A- 2019 531 413

## Description

### TECHNICAL FIELD

This disclosure relates to a hot pressed member and a method of producing the same, and a coated steel sheet for hot press forming.

### BACKGROUND

Conventionally, most automotive undercarriage parts and automotive body structural parts are produced by press working steel sheets with certain strength. In recent years, there has been an eagerness to reduce the weight of automobile automotive body from the perspective of preserving the global environment, and efforts have been made to increase the strength of the steel sheets used and to reduce their thickness. However, when a steel sheet has higher strength, its press formability is deteriorated, and forming the steel sheet into the desired part shape is becoming more difficult.

To address these issues, a working technique called hot press forming has been proposed. Hot press forming uses a press mold having a die and a punch to process a heated steel sheet while quenching it simultaneously, to achieve both easier working and higher strength. Among others, Zn alloy-coated steel sheets have attracted attention as steel sheets for hot press forming having high rust resistance since their coated layers, which are electrochemically more basic (with a lower potential) than the base steel sheets, remain after heating. Accordingly, hot pressed members using such Zn alloy-coated steel sheets and manufacturing methods thereof have been proposed in the art.

JP 2006-265706 A (PTL 1) describes a coated steel sheet for hot press forming having a coated layer in which an Al concentration {Al} is in the range of 0.2 g/m² to 1.0 g/m² and a Mg concentration {Mg} in mass % satisfies a relation with the Al concentration of 0.10 ≤ {Mg}/{Al} ≤ 5, and a hot pressed member obtained by heating the coated steel sheet for hot press forming and then subjecting it to hot press forming.
WO 2014/122900 A1 (PTL 2) describes a surface treatment liquid for a galvanized steel sheet that: is characterized by containing a zirconium carbonate compound (A), a phosphate compound (B), hydroxy carboxylic acid (C), tetra-alkoxysilane (D), a silane coupling agent (E) having an epoxy group, a vanadate compound (F), and a nickel compound (G); and is further characterized in that the contents of (A) to (G) are adjusted so as to satisfy specific conditions.
JP 2013-241671 A (PTL 3) describes a Zn-plated steel sheet having a Zn-plated layer containing molten Al and Mg. The Zn-plated layer containing molten Al and Mg includes 0.1-22.0 mass% of Al and 0.1-1.5 mass% of Mg. The plated layer is blackened by making the molten-plated steel sheet contact with water vapor in a tightly sealed container. At this time, the concentration of oxygen in the tightly sealed container is 13% or less.

### CITATION LIST

### Patent Literature

[PTL 1] JP 2006-265706 A
[PTL 2] WO 2014/122900 A1
[PTL 3] JP 2013-241671 A

### SUMMARY

### (Technical Problem)

PTL 1 describes that the hot pressed member has good post-painting corrosion resistance when subjected to electrodeposition painting (also called electrodeposition coating) after zinc phosphate-based chemical conversion treatment. In recent years, zirconium-based chemical conversion treatment has begun to replace the conventional zinc phosphate-based chemical conversion treatment. As such, hot pressed members are also increasingly required to have proper painting layer adhesion and post-painting corrosion resistance when subjected to electrodeposition painting after zirconium-based chemical conversion treatment. However, our examination revealed that although the hot pressed member described in PTL 1 has good post-painting corrosion resistance when subjected to electrodeposition painting after zinc phosphate-based chemical conversion treatment, it has insufficient painting layer adhesion and post-painting corrosion resistance when subjected to electrodeposition painting after zirconium-based chemical conversion treatment.

It would thus be helpful to provide a hot pressed member with excellent painting layer adhesion and post-painting corrosion resistance when subjected to electrodeposition painting after zirconium-based chemical conversion treatment, and a suitable method of producing the same.

It would also be helpful to provide a coated steel sheet for hot press forming that is suitably used as a material to obtain such hot pressed member.

### (Solution to Problem)

In order to address the above issues, the present inventors conducted a diligent study and made the following findings.

It is possible to improve the painting layer adhesion and post-painting corrosion resistance of a hot pressed member when subjected to electrodeposition painting after zirconium-based chemical conversion treatment, by restricting precipitation of a Γ phase, which is formed from an electrochemically basic intermetallic compound such as an Fe3Zn10 phase, in an Fe-Zn-Al-Mg-based alloy coated layer of the hot pressed member, and by increasing the total concentration of Al and Mg in a Zn-Al-Mg-containing oxide layer formed on the coated layer.

To produce such a hot pressed member having an Fe-Zn-Al-Mg-based alloy coated layer with a small amount of Γ-phase precipitation and an oxide layer with a large sum of Al and Mg concentrations, it is necessary to heat a coated steel sheet for hot press forming having a Zn-Al-Mg-based alloy coated layer with certain amounts of Al and Mg and a liquidus temperature of 400 °C or lower to a relatively low temperature before subjecting it to hot press forming.

Based on these discoveries, we provide the following.
[1] A hot pressed member according to claim 1.
[2] A method of producing the aforementioned hot press member, in accordance with claim 2.

### (Advantageous Effect)

The hot pressed member according to the present disclosure has excellent painting layer adhesion and post-painting corrosion resistance when subjected to electrodeposition painting after zirconium-based chemical conversion treatment. In addition, the method of producing a hot pressed member according to the present disclosure enables the production of a hot pressed member with excellent painting layer adhesion and post-painting corrosion resistance when subjected to electrodeposition painting after zirconium-based chemical conversion treatment.

The coated steel sheet for hot press forming according to the present disclosure is suitably used as a raw material for producing a hot pressed member with excellent painting layer adhesion and post-painting corrosion resistance when subjected to electrodeposition painting after zirconium-based chemical conversion treatment.

### BRIEF DESCRIPTION OF THE DRAWINGS

In the accompanying drawings:
FIG. 1 is a scanning electron microscope (SEM) micrograph of a cross-section of an Fe-Zn-Al-Mg-based alloy coated layer of a hot pressed member in No. 2 representing one of our examples; and
FIG. 2 is an SEM micrograph of a cross-section of an Fe-Zn-Al-Mg-based alloy coated layer of a hot pressed member in No. 8 representing one of comparative examples.

### DETAILED DESCRIPTION

### (Hot Pressed Member)

A hot pressed member according to one of the embodiments disclosed herein comprises: a base steel sheet; an Fe-Zn-Al-Mg-based alloy coated layer formed on at least one surface of the base steel sheet; and an oxide layer formed on the Fe-Zn-Al-Mg-based alloy coated layer.

### [Base Steel Sheet]

Although the base steel sheet of the hot pressed member in this embodiment is not limited to a particular steel sheet, it is preferable to use a steel sheet having the chemical composition as described in the section "(Coated Steel Sheet for Hot Press Forming)" below, in order for the resulting hot pressed member to have a tensile strength TS of 1470 MPa or more.

### [Fe-Zn-Al-Mg-based Alloy Coated Layer]

The Fe-Zn-Al-Mg-based alloy coated layer in the hot pressed member in this embodiment contains, preferably consists of, an α-Fe phase and a Γ phase.

The α-Fe phase is a solid solution phase that is mainly composed of Fe and contains Zn, Al, and Mg. When a coated steel sheet for hot press forming with a Zn-Al-Mg-based alloy coated layer is subjected to hot press forming, Zn, Al, and Mg in the coated layer diffuse into the base steel sheet and, in this diffusion region, a solid solution phase (α-Fe phase) mainly composed of Fe and containing Zn, Al, and Mg is formed. The α-Fe phase is formed so as to erode the surface layer of the base steel sheet of the coated steel sheet. However, in a hot pressed member, the α-Fe phase is generally interpreted to be part of the Fe-Zn-Al-Mg-based alloy coated layer located on the base steel sheet.

The Γ phase is a phase formed from an intermetallic compound that is mainly composed of Zn and contains Al, Mg, and Fe. Primarily, the Γ phase is composed of Fe3Zn10 phase. In this respect, Γ1 phase has a crystal structure similar to that of Γ phase and is difficult to distinguish by X-ray diffraction. Thus, as used herein, "Γ phase" is intended to include Γ1 phase. Other compositional intermetallic compounds that make up the Γ phase include, for example, Fe4Zn9, FeZn4, and Fe5Zn21. During hot press forming, the Zn-Al-Mg-based alloy coated layer that remains without contributing to diffusion into the base steel sheet incorporates Fe diffused from the base steel sheet, forming a Γ phase composed of an intermetallic compound and forming a part of the Fe-Zn-Al-Mg-based alloy coated layer in the hot pressed member.

The α-Fe and Γ phases can be distinguished from each other by their distinctly different contrasts in the cross-sectional SEM images of the Fe-Zn-Al-Mg-based alloy coated layer of the hot pressed member. Referring to FIGS. 1 and 2, regions that appear relatively bright in the surface layer of the hot pressed member are the Γ phase, and regions that appear relatively dark are the α-Fe phase. The α-Fe and Γ phases can also be identified using a Co-Kα (wavelength: 1.79021 Å) radiation source at an incident angle of 25°.

The Γ phase in the Fe-Zn-Al-Mg-based alloy coated layer has a significantly lower potential than the base steel sheet and the α-Fe phase, and is therefore preferentially corroded when exposed to a corrosion environment. In other words, the Γ phase provides sacrificial protection against the base steel sheet and the α-Fe phase.

A zinc phosphate-based chemical conversion treatment layer functions as an excellent corrosion inhibitor against Zn-based alloys. Therefore, when a hot pressed member obtained by subjecting a Zn-Al-Mg-based alloy-coated steel sheet to hot press forming is subjected to electrodeposition painting after zinc phosphate-based chemical conversion treatment, the resulting member has a low corrosion rate in the Γ phase and a sufficiently low corrosion rate under the painting layer such that post-painting corrosion resistance is not an issue in actual use environments even in a sacrificial protection state due to flaws that penetrate the painting layer, the chemical conversion treatment layer, and the coated layer to reach the base steel sheet.

In contrast, a zirconium oxide-based chemical conversion treatment layer does not have a corrosion inhibitor function against Zn-based alloys. Therefore, in a sacrificial protection state, the corrosion rate of the Γ phase becomes higher, resulting in a higher corrosion rate under the painting layer. Then, if a large amount of Γ phase is present contiguously in the Fe-Zn-Al-Mg-based alloy coated layer, corrosion in the Γ phase propagates in-plane under the painting layer in a sacrificial protection state, resulting in problems in lowered esthetics such as poor appearance including swelling in the painting layer. Therefore, when applying a zirconium-based chemical conversion treatment, it is important to limit the amount of Γ phase to ensure post-painting corrosion resistance.

Therefore, in this embodiment, as one of the necessary conditions to improve the post-painting corrosion resistance when the hot pressed member is subjected to electrodeposition painting after zirconium-based chemical conversion treatment, it is important to suppress the precipitation of a Γ phase, which is formed from an electrochemically basic intermetallic compound such as an Fe3Zn10 phase. Specifically, it is important that a ratio of I_{Γ}/I_{α} is 0.5 or less when measured by X-ray diffraction using a Co-Kα (wavelength: 1.79021 Å) radiation source at an incident angle of 25°, where I_{Γ} is an intensity of a diffraction peak of (411) plane of the Γ phase present in an angular range of 41.5° ≤ 2Θ ≤ 43.0° and I_{α} is an intensity of a diffraction peak of (110) plane of the α-Fe phase present in an angular range of 51.0° ≤ 2Θ ≤ 52.0°. If I_{Γ}/I_{α} is greater than 0.5, the post-painting corrosion resistance is insufficient when the hot pressed member is subjected to electrodeposition painting after zirconium-based chemical conversion treatment. If I_{Γ}/I_{α} is 0.5 or less, the Γ phase is sufficiently broken up by the α-Fe phase in the Fe-Zn-Al-Mg-based alloy layer, and excellent post-painting corrosion resistance can be obtained when the hot pressed member is subjected to electrodeposition painting after zirconium chemical conversion treatment.

Since a smaller value of I_{Γ}/I_{α} is preferable, the lower limit is not limited. However, the value of I_{Γ}/I_{α} that is detected by measurement using X-ray diffraction as described above is usually 0.01 or more.

The measurement conditions for X-ray diffraction other than the incident angle and radiation source described above, which do not affect the ratio of I_{Γ}/I_{α}, can be adopted as described in the EXAMPLES section below.

### Coating Weight Per Surface: 40 g/m² to 400 g/m²

By setting the coating weight of the Fe-Zn-Al-Mg-based alloy coated layer of the hot pressed member to 40 g/m² to 400 g/m², it is possible to provide the hot pressed member with excellent corrosion resistance. If the coating weight is less than 40 g/m², it is not possible to provide the hot pressed member with the desired corrosion resistance. If the coating weight exceeds 400 g/m², the number of cracks crossing the coated layer becomes significantly larger due to the solidification and shrinkage of the coated layer after hot pressing, and the adhesion in the coated layer is greatly degraded. The coating weight of the coated layer of the hot pressed member is preferably 50 g/m² or more, and more preferably 60 g/m² or more. The coating weight of the coated layer of the hot pressed member is preferably 350 g/m² or less, and more preferably 300 g/m² or less.

As used herein, the "coating weight per surface of the Fe-Zn-Al-Mg-based alloy coated layer" of the hot pressed member is determined as follows. From each hot pressed member to be evaluated, three 48 mmφ samples are taken by punching. Then, in each sample, a non-evaluated surface opposite the one surface where the coating weight is evaluated is masked. First, the oxide layer is dissolved by immersing each sample in a 20 % chromium oxide (VI) solution at room temperature for 10 minutes. Then, each sample is weighed. Next, 500 mL of a 35 % hydrochloric acid solution to which 3.5 g of hexamethylenetetetramine has been added is mixed up to 1 L. Then, each sample is immersed in the resultant solution for 120 minutes to dissolve the Fe-Zn-Al-Mg-based alloy coated layer. Then, each sample is weighed again. The coating weight per unit area in each sample is calculated from the mass difference before and after the dissolution of the Fe-Zn-Al-Mg-based alloy coated layer. The average of the three samples is then used as the coating weight per surface.

### [Oxide Layer]

The oxide layer of the hot pressed member in this embodiment is formed on the Fe-Zn-Al-Mg-based alloy coated layer and contains Zn, Al, and Mg. When a coated steel sheet for hot press forming with a Zn-Al-Mg-based alloy coated layer is subjected to hot press forming, Zn, Al, and Mg in the coated layer combine with oxygen present in the heating atmosphere to form an oxide layer containing Zn, Al, and Mg. The oxide layer is mainly composed of an Al oxide. However, it may also contain Zn and Mg contained in the coated layer, as well as elements constituting the base steel sheet, such as Fe, Mn, and Cr.

In this embodiment, as another necessary condition for improving the post-painting corrosion resistance when the hot pressed member is subjected to electrodeposition painting after zirconium-based chemical conversion treatment, it is important that the sum of the Al and Mg concentrations in the oxide layer be 28 atomic% or more. If the sum of the Al and Mg concentrations in the oxide layer is less than 28 atomic%, even with the ratio of I_{Γ}/I_{α} being 0.5 or less, the post-painting corrosion resistance is insufficient when the hot pressed member is subjected to electrodeposition painting after zirconium-based chemical conversion treatment. This is presumably because when the concentration of Zn constituting the oxide layer is high, the reaction between the chemical conversion treatment liquid and the oxide layer becomes non-uniform, resulting in a larger unevenness in the thickness of the zirconium-based chemical conversion treatment layer formed on the surface of the oxide layer. In other words, it is assumed that regions where the chemical conversion treatment layer becomes thin are formed more easily, resulting in reduced adhesion either between the oxide layer and the chemical conversion treatment layer or between the chemical conversion treatment layer and the painting layer, or incomplete coverage by the chemical conversion treatment layer. In contrast, if the sum of the Al and Mg concentrations in the oxide layer is 28 atomic% or more, a zirconium-based chemical conversion treatment layer is appropriately formed, and the hot pressed member may have excellent post-painting corrosion resistance when subjected to electrodeposition painting after zirconium-based chemical conversion treatment.

If the sum of the Al and Mg concentrations in the oxide layer is less than 28 atomic%, the oxide layer becomes brittle, resulting in insufficient painting layer adhesion when the hot pressed member is subjected to electrodeposition painting after the zirconium-based chemical conversion treatment. In contrast, if the sum of the Al and Mg concentrations in the oxide layer is 28 atomic% or more, the oxide layer has sufficient strength, and the hot pressed member has good painting layer adhesion when subjected to electrodeposition painting after zirconium-based chemical conversion treatment.

The upper limit of the sum of the Al and Mg concentrations in the oxide layer is not particularly limited. However, an oxide layer containing excessively high concentrations of Al and Mg is chemically stable in acidic environments, such as in a chemical conversion treatment liquid for coating base treatment, and may prevent the formation of a chemical conversion treatment layer. Therefore, the sum of the Al and Mg concentrations in the oxide layer is preferably 50 atomic% or less.

In this embodiment, the oxide layer is formed very thinly on the Fe-Zn-Al-Mg-based alloy coated layer, and thus may not be visible in the cross-sectional SEM image as illustrated in FIG. 1. However, by cross-sectioning the surface layer of the hot pressed member using energy dispersive X-ray analysis (EDX) combined with SEM, elemental mapping can be performed to identify the oxide layer as a region where oxygen is detected. As used herein, "the Al and Mg concentrations in the oxide layer" are the values measured by the following methods. Specifically, a test specimen for cross-sectional observation is taken from a flat part of the hot pressed member. A cross-section of the test specimen including the Fe-Zn-Al-Mg-based alloy coated layer and the oxide layer is observed under SEM at 10000x magnification and accelerating voltage of 15 kV, and the composition of the oxide layer is measured at freely-selected three locations using EDX. The arithmetic means of the Al concentrations and Mg concentrations at the three locations are respectively used as the "Al concentration in the oxide layer" and "Mg concentration in the oxide layer".

### (Method of Producing the Hot Pressed Member)

A method of producing the hot pressed member according to one of the embodiments of the present disclosure comprises: heating a coated steel sheet for hot press forming according to one of the embodiments of the present disclosure as described below to a temperature range of Ac₃ transformation point to 1000 °C; and then subjecting the coated steel sheet to hot press forming.

By setting the heating temperature of the steel sheet for hot press forming before hot press forming to the temperature range of Ac₃ transformation point to 1000 °C, it is possible to obtain an Fe-Zn-Al-Mg-based alloy coated layer with α-Fe and Γ phases as well as an oxide layer with predetermined Al and Mg concentrations, as described above. When the heating temperature is lower than the Ac₃ transformation point, the I_{Γ}/I_{α} of the Fe-Zn-Al-Mg-based alloy coated layer exceeds 0.5 after hot press forming. Consequently, the post-painting corrosion resistance becomes insufficient when the hot pressed member is subjected to electrodeposition painting after zirconium-based chemical conversion treatment. If the heating temperature exceeds 1000 °C, the desired oxide layer cannot be obtained, and the painting layer adhesion and post coating corrosion resistance are insufficient when the hot pressed member is subjected to electrodeposition painting after zirconium-based chemical conversion treatment. As used herein, the "heating temperature" refers to the maximum arrival temperature of the steel sheet. As used herein, " Ac₃ transformation point" is a value calculated from the following formula based on the chemical composition of the steel sheet: ${Ac}_{3} transformation point \left(°C\right) = 910 - 203 {C}^{1 / 2} + 44.7 Si - 4 Mn + 11 Cr .$ The element symbols on the right side of the formula indicate the content of each element. When Cr is not contained, Cr = 0.

The holding time after the temperature is raised to the heating temperature is 30 seconds or longer from the viewpoint of eliminating the Γ phase and avoiding liquid metal embrittlement cracking during hot press forming. From the perspective of avoiding hydrogen ingress due to the inclusion of water vapor present in the furnace during the holding time, the holding time is within 5 minutes, preferably within 3 minutes, and more preferably within 2 minutes.

The method of heating the steel sheet for hot press forming is not limited in any way, and exemplary methods include furnace heating such as heating in an electric or gas furnace, electrical resistance heating, induction heating, high-frequency heating, and flame heating.

In hot press forming, the coated steel sheet for hot press forming heated as described above is simultaneously subjected to press forming and quenching using a press forming tool to obtain a hot pressed member of a predetermined shape. The conditions for hot press forming are not limited, and conventional methods may be followed.

### (Coated Steel Sheet for Hot Press Forming)

The coated steel sheet for hot press forming according to one of the embodiments of the present disclosure comprises: a base steel sheet; and a Zn-Al-Mg-based alloy coated layer formed on at least one surface of the base steel sheet at a coating weight per surface of 30 g/m² to 180 g/m², having a chemical composition containing, in mass%, Al: 3 % to 10 % and Mg: 0.2 % to 0.8 %, with the balance being Zn and inevitable impurities, and having a liquidus temperature in an air atmosphere of 400 °C or lower.

### [Base Steel Sheet]

To obtain a hot pressed member having a tensile strength TS of 1470 MPa or more, the base steel sheet has a chemical composition containing, in mass%, C: 0.20 % to 0.35 %, Si: 0.1 % to 0.5 %, Mn: 1.0 % to 3.0 %, P: 0.1 % or less, S: 0.05 % or less, Al: 0.1 % or less, N: 0.01 % or less, with the balance being Fe and inevitable impurities. The base steel sheet may be a cold-rolled steel sheet or a hot-rolled steel sheet.
The reasons for the limitation of each component will be explained below.

### C: 0.20 % to 0.35 %

C increases strength by forming a steel microstructure such as martensite. To obtain a TS of 1470 MPa or more, the C content needs to be 0.20 % or more. However, if the C content exceeds 0.35 %, the toughness deteriorates at a spot welded portion. Therefore, the C content is preferably 0.20 % to 0.35 %.

### Si: 0.1 % to 0.5 %

Si is an effective element in increasing the strength of steel to obtain good material properties. To this end, the Si content needs to be 0.1 % or more. However, if the Si content exceeds 0.5 %, ferrite is stabilized and hardenability is reduced. Therefore, the Si content is preferably 0.1 % to 0.5 %.

### Mn: 1.0 % to 3.0 %

Mn is an effective element for increasing the strength of steel. To ensure proper mechanical properties and strength, the Mn content needs to be 1.0 % or more. However, if the Mn content exceeds 3.0 %, surface enrichment during annealing becomes more pronounced, making it difficult to ensure proper coating adhesion. Therefore, the Mn content is preferably 1.0 % to 3.0 %.

### P: 0.1 % or less

If the P content exceeds 0.1 %, the balance between strength and ductility is reduced as a result of degradation in local ductility due to grain boundary embrittlement caused by P segregation at austenite grain boundaries during casting. Therefore, the P content is preferably 0.1 % or less. From the viewpoint of steelmaking cost, the P content is preferably 0.01 % or more.

### S: 0.05 % or less

S forms as inclusions such as MnS, which cause degradation of impact resistance and cracking along the metal flow in welded portions. Therefore, a lower S content is desirable, and the S content is preferably 0.05 % or less. To ensure good stretch flangeability, the S content is more preferably 0.01 % or less. From the viewpoint of steelmaking cost, the S content is preferably 0.002 % or more.

### Al: 0.1 % or less

If the Al content exceeds 0.1 %, the blanking workability and hardenability of the base steel sheet decrease. Therefore, the Al content is preferably 0.1 % or less. From the viewpoint of ensuring its effectiveness as a deoxidizing material, the Al content is preferably 0.01 % or more.

### N: 0.01 % or less

If the N content exceeds 0.01 %, AlN is formed during hot rolling or heating before hot press forming, and the blanking workability and hardenability of the base steel sheet decrease. Therefore, the N content is preferably 0.01 % or less. From the viewpoint of steelmaking cost, the N content is preferably 0.001 % or more.

The balance other than the above elements is Fe and inevitable impurities. However, the chemical composition may optionally contain at least one selected from the group consisting of Nb: 0.05 % or less, Ti: 0.05 % or less, B: 0.0002 % to 0.005 %, Cr: 0.1 % to 0.3 %, Sb: 0.003 % to 0.03 %, for the reasons given below.

### Nb: 0.05 % or less

Nb is an effective component for increasing the strength of steel. However, excessive addition of Nb reduces shape fixability. Therefore, when Nb is contained, the Nb content is 0.05 % or less.

### Ti: 0.05 % or less

As in Nb, Ti is also effective in increasing the strength of steel. However, excessive addition of Ti reduces shape fixability. Therefore, when Ti is contained, the Ti content is 0.05 % or less.

### B: 0.0002 % to 0.005 %

B has an effect of inhibiting the formation and growth of ferrite from austenite grain boundaries. Therefore, the B content is preferably 0.0002 % or more. However, excessive addition of B greatly impairs formability. Therefore, when B is contained, the B content is 0.005 % or less.

### Cr: 0.1 % to 0.3 %

Cr is useful for increasing the strength and hardenability of steel. To obtain this effect, the Cr content is preferably 0.1 % or more. However, from the viewpoint of alloy cost, when Cr is contained, the Cr content is 0.3 % or less.

### Sb: 0.003 % to 0.03 %

Sb has an effect of deterring decarburization of the surface layer of the steel sheet during hot pressing. To obtain this effect, the Sb content is preferably 0.003 % or more. However, if the Sb content exceeds 0.03 %, the rolling load increases, resulting in lower productivity. Therefore, when Sb is contained, the Sb content is 0.03 % or less.

### [Zn-Al-Mg-based Alloy Coated Layer]

In this embodiment, the Zn-Al-Mg-based alloy coated layer of the coated steel sheet for hot press forming has a chemical composition containing, in mass%, Al: 3 % to 10 % and Mg: 0.2 % to 0.8 %, with the balance being Zn and inevitable impurities, and has a liquidus temperature in an air atmosphere of 400 °C or lower.

### Al: 3 % to 10 %

If the Al content is less than 3 %, the I_{Γ}/I_{α} of the Fe-Zn-Al-Mg-based alloy coated layer exceeds 0.5 after hot press forming, and the sum of the Al and Mg concentrations in the oxide layer is less than 28 atomic%. As a result, the painting layer adhesion and post-painting corrosion resistance are insufficient when the hot pressed member is subjected to electrodeposition painting after zirconium-based chemical conversion treatment. If the Al content is less than 3 %, depending on the Mg content, the liquidus temperature to be described later cannot be lowered to 400 °C or lower. On the other hand, if the Al content exceeds 10 %, the liquidus temperature to be described later cannot be lowered to 400 °C or lower, with the result that the I_{Γ}/I_{α} of the Fe-Zn-Al-Mg-based alloy coated layer exceeds 0.5 after hot press forming. Consequently, the post-painting corrosion resistance becomes insufficient when the hot pressed member is subjected to electrodeposition painting after zirconium-based chemical conversion treatment. Therefore, the Al content is 3 % to 10 %.

### Mg: 0.2 % to 0.8 %

When the Mg content is less than 0.2 %, the I_{Γ}/I_{α} of the Fe-Zn-Al-Mg-based alloy coated layer exceeds 0.5 after hot press forming. Consequently, the post-painting corrosion resistance becomes insufficient when the hot pressed member is subjected to electrodeposition painting after zirconium-based chemical conversion treatment. Therefore, the Mg content is 0.2 % or more, preferably 0.3 % or more, and more preferably 0.4 % or more. However, if the Mg content exceeds 0.8 %, the sum of the Al and Mg concentrations in the oxide layer is less than 28 atomic% after hot press forming. Consequently, the painting layer adhesion and post-painting corrosion resistance becomes insufficient when the hot pressed member is subjected to electrodeposition painting after zirconium-based chemical conversion treatment. Therefore, the Mg content is 0.8 % or less, preferably 0.7 % or less, and more preferably 0.6 % or less.

### Liquidus Temperature in Air Atmosphere: 400 °C or lower

In this embodiment, it is important to keep the liquidus temperature of the Zn-Al-Mg-based alloy coated layer in an air atmosphere at or below 400°C by controlling the Al and Mg contents as appropriate. If the liquidus temperature is above 400 °C, the I_{Γ}/I_{α} of the Fe-Zn-Al-Mg-based alloy coated layer exceeds 0.5 after hot press forming. Consequently, the post-painting corrosion resistance becomes insufficient when the hot pressed member is subjected to electrodeposition painting after zirconium-based chemical conversion treatment. The lower limit of the liquidus temperature is not particularly limited, yet in the range of Al and Mg contents specified above, the liquidus temperature is generally 380 °C or higher. The liquidus temperatures of the Zn-Al-Mg-based alloy coated layer in an air atmosphere are calculated by Thermo Calc, a thermodynamic calculation software, using a database.

The inevitable impurities contained in the Zn-Al-Mg-based alloy coated layer include components of the base steel sheet that are incorporated into the coated layer by the reaction between the coating bath and the base steel sheet during the coating treatment, inevitable impurities in the coating bath, and so on. The components of the base steel sheet that are incorporated into the coated layer include Fe in an amount of 0.01 % to several percent. The inevitable impurities in the coating bath include, for example, Fe, Cr, Cu, Mo, Ni, and Zr. As to Fe in the coated layer, it is not possible to quantify the amount of Fe incorporated from the base steel sheet and the amount of Fe incorporated from the coating bath separately. Although the total content of inevitable impurities is not limited, from the viewpoint of uniform melting of the coated layer during the process of hot press forming, the total amount of inevitable impurities, excluding Fe, is preferably 1 mass% or less.

The chemical composition of the Zn-Al-Mg-based alloy coated layer may further contain at least one selected from the group consisting of Ca, Sr, Mn, V, Cr, Mo, Ti, Ni, Co, Sb, Zr, and B in a total amount of 1 mass% or less.

### Coating Weight Per Surface: 30 g/m² to 180 g/m²

By setting the coating weight of the Zn-Al-Mg-based alloy coated layer in the range of 30 g/m² to 180 g/m², it is possible to obtain a hot pressed member that is excellent in corrosion resistance and resistance to liquid metal embrittlement cracking during hot press forming. If the coating weight is less than 30 g/m², it is not possible to obtain a hot pressed member with the desired corrosion resistance. If the coating weight exceeds 180 g/m², alloying is not completed in the heating process before hot press forming, and the liquid phase remains. This may cause liquid metal embrittlement cracking. The coating weight of the Zn-Al-Mg-based alloy coated layer is preferably 45 g/m² or more, and more preferably 55 g/m² or more. The coating weight of the Zn-Al-Mg-based alloy coated layer is preferably 120 g/m² or less, and more preferably 100 g/m² or less.

As used herein, the "coating weight per surface of the Zn-Al-Mg-based alloy coated layer" is determined as follows. From each of the Zn-Al-Mg alloy-coated steel sheets to be evaluated, three 48 mmφ samples are taken by punching. Then, each sample is weighed. Subsequently, in each sample, a non-evaluated surface opposite the one surface where the coating weight is evaluated is masked. Then, 500 mL of a 35 % hydrochloric acid solution to which 3.5 g of hexamethylenetetetramine has been added is mixed up to 1 L. Then, each sample is immersed in the resultant solution for 10 minutes to dissolve the Zn-Al-Mg-based alloy coated layer. Then, each sample is weighed again. The coating weight per unit area in each sample is calculated from the mass difference before and after the dissolution of the Zn-Al-Mg-based alloy coated layer. The average of the three samples is then used as the coating weight per surface.

In this embodiment, as a lower or upper layer of the Zn-Al-Mg-based alloy coated layer, an additional layer may be provided according to the purpose without deteriorating the actions and effects of the present disclosure. Examples of the lower layer include a nickel pre-coated layer. Examples of the upper layer include a chemical conversion treatment layer containing, for example, a zirconium oxide or a zirconium-titanium oxide.

### EXAMPLES

The base steel sheets used were cold-rolled steel sheets (Ac₃ = 814 °C) of 1.4 mm thick, each having a chemical composition containing, in mass%, C: 0.23 %, Si: 0.25 %, Mn: 1.2 %, P: 0.005 %, S: 0.001 %, Al: 0.03 %, N: 0.004 %, Nb: 0.02 %, Ti: 0.02 %, B: 0.002 %, Cr: 0.2 %, and Sb: 0.008 %, with the balance being Fe and inevitable impurities.

The cold-rolled steel sheets were immersed in a hot-dip Zn-Al-Mg-based coating bath with a predetermined chemical composition at a predetermined bath temperature in a galvanizing line, and then subjected to N₂ gas wiping, to produce coated steel sheets for hot press forming, which are labeled No. 1 to No. 14 in Table 1. Table 1 lists the Al content, the Mg content, and the content of other elements, as well as the liquidus temperature in an air atmosphere for each Zn-Al-Mg-based alloy coated layer. The content of each element and the liquidus temperature were controlled by adjusting the chemical composition of the coating bath. The content of each element in the coated layer was determined by quantitative analysis of each component of the coated layer contained in the hydrochloric acid exfoliation solution using ICP-AES. The liquidus temperature of the coated layer was determined by the above-mentioned method. Table 1 also lists the coating weight per surface of the Zn-Al-Mg-based alloy coated layer as determined by the above-described method. The coating weight was controlled by adjusting the wiping gas flow rate and the line speed.

Then, the steel sheets for hot press forming thus obtained were subjected to hot press forming. Specifically, from each obtained steel sheet for hot press forming, a test specimen of 150 mm × 300 mm was taken and subjected to heat treatment in an electric furnace. The heat treatment conditions (heating temperature and holding time) are listed in Table 1. After the heat treatment, each test specimen was removed from the electric furnace and immediately subjected to hot press forming at a forming start temperature of 700 °C using a hat-shaped press mold to obtain a hot pressed member. The shape of each obtained hot pressed member was 100 mm in flat length on the top surface, 50 mm in flat length on the side surfaces, and 50 mm in flat length on the bottom surface. The bending radius (or bending R) of the press mold was 7R for each shoulder on both the top and bottom surfaces.

### (Evaluation of Fe-Zn-Al-Mg-based Alloy Coated Layer/Oxide layer of Hot Pressed Member)

From a flat part on the top surface of each obtained hot pressed member, a test specimen was taken for cross-sectional observation, and a cross-section of the Fe-Zn-Al-Mg-based alloy coated layer was observed under SEM. In each sample, α-Fe and Γ phases could be distinguished from each other by their distinctly different contrasts in the cross-sectional SEM image. FIG. 1 illustrates a cross-sectional SEM image of the Fe-Zn-Al-Mg-based alloy coated layer of the hot pressed member indicated by No. 2, which represents one of our examples, and FIG. 2 illustrates a cross-sectional SEM image of the Fe-Zn-Al-Mg-based alloy coated layer of the hot pressed member indicated by No. 8, which represents one of comparative examples. In FIG. 1, precipitation of the Γ phase is suppressed, and the Γ phase is scattered discontinuously in the α-Fe phase. In contrast, in FIG. 2, precipitation of the Γ phase is more significant, and the Γ phase is present in the form of continuous planes. In addition, I_{Γ} and I_{α} were measured by X-ray diffraction using a Co-Kα (wavelength: 1.79021 Å) radiation source at an incident angle of 25°, where I_{Γ} is an intensity of a diffraction peak of (411) plane of the Γ phase present in an angular range of 41.5° ≤ 2θ ≤ 43.0° and I_{α} is an intensity of a diffraction peak of (110) plane of the α-Fe phase present in an angular range of 51.0° ≤ 2θ ≤ 52.0°. Table 1 lists the ratio of I_{Γ}/I_{α}. X-ray diffraction measurements were performed using a curved IP X-ray diffractometer (RINT-RAPID II-R available from Rigaku Corporation), under a set of conditions including tube voltage of 45 kV, tube current of 160 mA, integration time of 600 sec, and collimator diameter of 3 mm.

For each sample, the Al and Mg concentrations in the oxide layer were measured by the above-mentioned method, and the results are listed in Table 1. In addition, for each sample, the coating weight per surface of the Fe-Zn-Al-Mg-based alloy coated layer was measured by the above-mentioned method, and the results are listed in Table 1.

### (Evaluation 1: Painting Layer Adhesion)

A test specimen of 70 mm × 150 mm was cut from a flat part on the top surface of each obtained hot pressed member, and subjected to zirconium-based chemical conversion treatment. Specifically, the chemical conversion treatment was performed using commercially available chemical conversion treatment liquid (zirconium-based chemical conversion treatment: Palmina 2100, available from Nihon Parkerizing Co. Ltd.) under a set of conditions including bath temperature of 35°C and treatment time of 120 seconds. Then, each test specimen was energized under the voltage condition that the voltage was raised in 30 seconds and held at a constant voltage for 150 seconds such that a painting layer having a thickness of 1.5 µm would be formed after baking with commercially available cationic electrodeposition paint, and then baked in an electric furnace at an ambient temperature of 170 °C for 20 minutes. The cationic electrodeposition paint used was Electron GT-100 V-1 Gray, available from Kansai Paint Co. Ltd.

Eleven cuts reaching the base steel sheet were made on each test specimen after electrodeposition painting with a cutter knife at intervals of 1 mm in each of the longitudinal and transverse directions to make one hundred grid squares on a surface of the test specimen. The cellophane tape^{®} ("cellophane tape" is a registered trademark in Japan, other countries, or both) was strongly pressed onto the grid, and the edge of the tape was pulled off at once at a 45° angle. The number of grid squares of the painting layer that were peeled off from the surface of each test specimen was counted and judged according to the criteria shown below, with Excellent or Good being accepted. The evaluation results are presented in Table 1.

| | |
|---|---|
| Excellent: | the number of grid squares peeled off = 0 |
| Good: | the number of grid squares peeled off = 1 |
| Fair: | the number of grid squares peeled off = 2 to 5 |
| Poor: | the number of grid squares peeled off = more than 5 |

### (Evaluation 2: Post-painting Corrosion Resistance)

Test specimens were prepared in the same way as in Evaluation 1 until the step of electrodeposition painting, and the 7.5 mm edge of the evaluation surface and the non-evaluation surface (rear side) of each test specimen were sealed with tape. Then, a cross-cut scratch of 60 mm in length and 60° center angle was made in the center of the evaluation surface with a cutter knife to a depth that reached the base steel sheet. Each obtained test specimen was subjected to a corrosion test (VDA 233-102) and evaluated according to the corrosion condition after 4 weeks.

The maximum swelling width on one side from the crosscut was measured and judged according to the criteria shown below, with Excellent or Good being accepted. The evaluation results are presented in Table 1.

| | |
|---|---|
| Excellent: | maximum swelling width on one side = less than 1.5 mm |
| Good: | maximum swelling width on one side = 1.5 mm or more and less than 3.0 mm |
| Fair: | maximum swelling width on one side = 3.0 mm or more and less than 4.0 mm |
| Poor: | maximum swelling width on one side = 4.0 mm or more |

**Table 1**

| No. | Steel sheet for hot press forming | | | | | | Heating before hot press forming | | Hot pressed member | | | Evaluation results | | Classification |
|---|---|---|---|---|---|---|---|---|---|---|---|---|---|---|
| | Coated layer | | | | | Steel sheet | Heating temp. (°C) | Holding time (mill) | Coated layer | | Oxide layer | Painting layer adhesion | Post-painting corrosion resistance | |
| | Al content (mass%) | Mg content (mass%) | Optional element (mass%) | Liquidus temp. (°C) | Coating weight (g/m²) | Ac₃ Transformation point (°C) | | | I_{Γ}/I_{α} | Coating weight (g/m²) | Al + Mg (atomic%) | | | |
| 1 | 4 | 0.3 | - | 383 | 60 | 814 | 800 | 1 | 0.8 | 90 | 30 | Excellent | Fair | Comparative Example |
| 2 | 4 | 0.3 | - | 383 | 60 | 814 | 950 | 1 | 0.3 | 180 | 37 | Excellent | Excellent | Example |
| 3 | 4 | 0.3 | - | 383 | 60 | 814 | 950 | 5 | 0.1 | 240 | 30 | Good | Excellent | Example |
| 4 | 4 | 0.3 | - | 383 | 60 | 814 | 1050 | 5 | 0.1 | 600 | 15 | Poor | Poor | Comparative Example |
| 5 | 4 | 0.3 | - | 383 | 90 | 814 | 950 | 1 | 0.4 | 270 | 37 | Excellent | Excellent | Example |
| 6 | 4 | 0.3 | - | 383 | 90 | 814 | 950 | 5 | 0.2 | 360 | 30 | Good | Excellent | Example |
| 7 | 4 | 0.3 | - | 383 | 35 | 814 | 950 | 1 | 0.1 | 70 | 42 | Excellent | Good | Example |
| 8 | 0.2 | 0.0 | - | 417 | 60 | 814 | 950 | 1 | 60 | 150 | 10 | Poor | Poor | Comparative Example |
| 9 | 7.5 | 0.3 | - | 405 | 60 | 814 | 950 | 1 | 0.6 | 180 | 35 | Excellent | Fair | Comparative Example |
| 10 | 6 | 0.7 | - | 385 | 60 | 814 | 950 | 1 | 0.3 | 180 | 31 | Excellent | Excellent | Example |
| 11 | 6 | 0.7 | Cr, 0.05 % | 385 | 60 | 814 | 950 | 1 | 0.3 | 180 | 35 | Excellent | Excellent | Example |
| 12 | 6 | 0.7 | Cr, 0.5 % | 385 | 60 | 814 | 950 | 1 | 0.3 | 180 | 40 | Excellent | Excellent | Example |
| 13 | 6 | 0.7 | Ni, 0.05 % | 385 | 60 | 814 | 950 | 1 | 0.3 | 180 | 35 | Excellent | Excellent | Example |
| 14 | 6 | 0.7 | Ni, 0.5 % | 385 | 60 | 814 | 950 | 1 | 0.3 | 180 | 40 | Excellent | Excellent | Example |

It can be seen from the results in Table 1 that each of the hot pressed members in our examples has excellent painting layer adhesion and post-painting corrosion resistance when subjected to electrodeposition painting after zirconium-based chemical conversion treatment.

### INDUSTRIAL APPLICABILITY

The hot pressed member according to the present disclosure is suitable for automotive undercarriage parts and automotive body structural parts.

## Claims

1. A hot pressed member comprising:
a base steel sheet having a chemical composition containing, in mass%, C: 0.20 % to 0.35 %, Si: 0.1 % to 0.5 %, Mn: 1.0 % to 3.0 %, P: 0.1 % or less, S: 0.05 % or less, Al: 0.1 % or less, and N: 0.01 % or less, optionally at least one selected from the group consisting of Nb: 0.05 % or less, Ti: 0.05 % or less, B: 0.0002 % to 0.005 %, Cr: 0.1 % to 0.3 %, and Sb: 0.003 % to 0.03 %, with the balance being Fe and inevitable impurities;
a Fe-Zn-Al-Mg-based alloy coated layer containing an α-Fe phase and a Γ phase and formed on at least one surface of the base steel sheet at a coating weight per surface of 40 g/m² to 400 g/m²; and
an oxide layer containing Zn, Al, and Mg and formed on the Fe-Zn-Al-Mg-based alloy coated layer, wherein
a ratio of I_{Γ}/I_{α} is 0.5 or less when measured by X-ray diffraction using a Co-Kα (wavelength: 1.79021 Å) radiation source at an incident angle of 25°, where Ir is an intensity of a diffraction peak of (411) plane of the Γ phase present in an angular range of 41.5° ≤ 2Θ ≤ 43.0° and I_{α} is an intensity of a diffraction peak of (110) plane of the α-Fe phase present in an angular range of 51.0° ≤ 2Θ ≤ 52.0°, and
a sum of Al and Mg concentrations in the oxide layer is 28 atomic% or more,
wherein the coating weight per surface of the Fe-Zn-Al-Mg-based alloy coated layer is determined in accordance with the description.

2. A method of producing a hot pressed member, the method comprising:
heating a coated steel sheet for hot press forming to a temperature range of Ac₃ transformation point to 1000 °C, wherein the holding time after the temperature is raised to the heating temperature is 30 seconds or longer and within 5 minutes, the coated steel sheet for hot press forming comprising:
a base steel sheet having a chemical composition containing, in mass%, C: 0.20 % to 0.35 %, Si: 0.1 % to 0.5 %, Mn: 1.0 % to 3.0 %, P: 0.1 % or less, S: 0.05 % or less, Al: 0.1 % or less, and N: 0.01 % or less, optionally at least one selected from the group consisting of Nb: 0.05 % or less, Ti: 0.05 % or less, B: 0.0002 % to 0.005 %, Cr: 0.1 % to 0.3 %, and Sb: 0.003 % to 0.03 %, with the balance being Fe and inevitable impurities; and
a Zn-Al-Mg-based alloy coated layer formed on at least one surface of the base steel sheet at a coating weight per surface of 30 g/m² to 180 g/m², having a chemical composition containing, in mass%, Al: 3 % to 10 % and Mg: 0.2 % to 0.8 %, and optionally containing at least one selected from the group consisting of Ca, Sr, Mn, V, Cr, Mo, Ti, Ni, Co, Sb, Zr, and B in a total amount of 1 mass% or less, with the balance being Zn and inevitable impurities, and having a liquidus temperature in an air atmosphere of 400 °C or lower, and
then subjecting the coated steel sheet to hot press forming to produce the hot pressed member according to claim 1,
wherein the coating weight per surface of the Zn-Al-Mg-based alloy coated layer is determined in accordance with the description.

## Patentansprüche

1. Heißgepresstes Bauteil, umfassend:
ein Basisstahlblech mit einer chemischen Zusammensetzung, die in Masse-% C: 0,20 % bis 0,35 %, Si: 0,1 % bis 0,5 %, Mn: 1,0 % bis 3,0 %, P: 0,1 % oder weniger, S: 0,05 % oder weniger, Al: 0,1 % oder weniger und N: 0,01 % oder weniger enthält, optional mindestens eines ausgewählt aus der Gruppe bestehend aus Nb: 0,05 % oder weniger, Ti: 0,05 % oder weniger, B: 0,0002 % bis 0,005 %, Cr: 0,1 % bis 0,3 % und Sb: 0,003 % bis 0,03 %, wobei der Restanteil aus Fe und unvermeidlichen Verunreinigungen besteht;
eine Beschichtungsschicht aus einer Legierung auf Fe-Zn-Al-Mg-Basis, die eine α-Fe-Phase und eine Γ-Phase enthält und auf mindestens einer Fläche des Basisstahlblechs mit einem Beschichtungsgewicht pro Fläche von 40 g/m² bis 400 g/m² gebildet ist; und
eine Oxidschicht, die Zn, Al und Mg enthält und auf der Beschichtungsschicht aus einer Legierung auf Fe-Zn-Al-Mg-Basis gebildet ist, wobei
ein Verhältnis von I_{Γ}/I_{α} 0,5 oder weniger beträgt, gemessen durch Röntgenbeugung unter Verwendung einer Co-Kα-Strahlungsquelle (Wellenlänge: 1,79021 Å) bei einem Einfallswinkel von 25°, wobei I_{Γ} die Intensität eines Beugungspeaks der (411)-Ebene der Γ-Phase in einem Winkelbereich von 41,5° ≤ 2θ ≤ 43,0° ist und I_{α} eine Intensität eines Beugungspeaks der (110)-Ebene der α-Fe-Phase in einem Winkelbereich von 51,0 ° ≤ 2θ ≤ 52,0° ist, und eine Summe der Al- und Mg-Konzentrationen in der Oxidschicht 28 Atom-% oder mehr beträgt,
wobei das Beschichtungsgewicht pro Fläche der beschichteten Schicht aus einer Legierung auf Fe-Zn-Al-Mg-Basis gemäß der Beschreibung bestimmt wird.

2. Verfahren zum Herstellen eines heißgepressten Bauteils, wobei das Verfahren Folgendes umfasst:
Erwärmen eines beschichteten Stahlblechs zum Heißpressformen auf einen Temperaturbereich vom Ac₃-Umwandlungspunkt bis 1000 °C, wobei die Haltezeit nach Erhöhung der Temperatur auf die Erwärmungstemperatur 30 Sekunden oder länger und innerhalb von 5 Minuten beträgt, wobei das beschichtete Stahlblech zum Heißpressumformen umfasst:
ein Basisstahlblech mit einer chemischen Zusammensetzung, die in Masse-% C: 0,20 % bis 0,35 %, Si: 0,1 % bis 0,5 %, Mn: 1,0 % bis 3,0 %, P: 0,1 % oder weniger, S: 0,05 % oder weniger, Al: 0,1 % oder weniger und N: 0,01 % oder weniger enthält, optional mindestens eines ausgewählt aus der Gruppe bestehend aus Nb: 0,05 % oder weniger, Ti: 0,05 % oder weniger, B: 0,0002 % bis 0,005 %, Cr: 0,1 % bis 0,3 % und Sb: 0,003 % bis 0,03 %, wobei der Restanteil aus Fe und unvermeidlichen Verunreinigungen besteht; und
eine Beschichtungsschicht aus einer Legierung auf Zn-Al-Mg-Basis, die auf mindestens einer Fläche des Basisstahlblechs mit einem Überzugsgewicht pro Fläche von 30 g/m² bis 180 g/m² gebildet ist und eine chemische Zusammensetzung aufweist, die in Masse-%: Al: 3 % bis 10 % und Mg: 0,2 % bis 0,8 % enthält und optional mindestens eines ausgewählt aus der Gruppe bestehend aus Ca, Sr, Mn, V, Cr, Mo, Ti, Ni, Co, Sb, Zr und B in einer Gesamtmenge von 1 Masse-% oder weniger enthält, wobei der Restanteil aus Zn und unvermeidlichen Verunreinigungen besteht und eine Liquidustemperatur in einer Luftatmosphäre von 400 °C oder weniger aufweist, und
anschließendes Unterziehen des beschichteten Stahlblechs einer Heißpressumformung, um das heißgepresste Bauteil gemäß Anspruch 1 herzustellen,
wobei das Beschichtungsgewicht pro Fläche der beschichteten Schicht aus einer Legierung auf Zn-Al-Mg-Basis gemäß der Beschreibung bestimmt wird.

## Revendications

1. Élément pressé à chaud comprenant :
une tôle d'acier de base ayant une composition chimique contenant, en % en masse, C : 0,20 % à 0,35 %, Si : 0,1 % à 0,5 %, Mn : 1,0 % à 3,0 %, P : 0,1 % ou moins, S : 0,05 % ou moins, Al : 0,1 % ou moins et N : 0,01 % ou moins, éventuellement au moins un élément choisi dans le groupe constitué de Nb : 0,05 % ou moins, Ti : 0,05 % ou moins, B : 0,0002 % à 0,005 %, Cr : 0,1 % à 0,3 %, et Sb : 0,003 % à 0,03 %, le reste étant constitué de Fe et d'impuretés inévitables ;
une couche revêtue d'un alliage à base de Fe-Zn-Al-Mg contenant une phase d'α-Fe et une phase Γ et formée sur au moins une surface de la tôle d'acier de base à un poids de revêtement par surface de 40 g/m² à 400 g/m² ; et
une couche d'oxyde contenant du Zn, de l'Al et du Mg et formée sur la couche revêtue d'un alliage à base de Fe-Zn-Al-Mg, dans lequel
un rapport I_{Γ}/I_{α} est de 0,5 ou moins lorsqu'il est mesuré par diffraction des rayons X à l'aide d'une source de rayonnement Kα de Co (longueur d'onde : 1,79021 Å) à un angle d'incidence de 25°, où I_{Γ} est une intensité d'un pic de diffraction du plan (411) de la phase Γ présent dans une plage angulaire de 41,5° ≤ 2θ ≤ 43,0° et I_{α} est une intensité d'un pic de diffraction du plan (110) de la phase d'α-Fe présent dans une plage angulaire de 51,0 ° ≤ 2θ ≤ 52,0°, et
une somme des concentrations d'Al et de Mg dans la couche d'oxyde est de 28 % atomique ou plus,
dans lequel le poids de revêtement par surface de la couche revêtue d'un alliage à base de Fe-Zn-Al-Mg est déterminé conformément à la description.

2. Procédé de production d'un élément pressé à chaud, le procédé comprenant :
le chauffage d'une tôle d'acier revêtue pour un formage par presse à chaud jusqu'à une plage de températures allant du point de transformation d'Ac₃ à 1 000 °C, dans lequel le temps de maintien après que la température a augmenté jusqu'à la température de chauffage est de 30 secondes ou plus et dans les 5 minutes, la tôle d'acier revêtue pour le formage par presse à chaud comprenant :
une tôle d'acier de base ayant une composition chimique contenant, en % en masse, C : 0,20 % à 0,35 %, Si : 0,1 % à 0,5 %, Mn : 1,0 % à 3,0 %, P : 0,1 % ou moins, S : 0,05 % ou moins, Al : 0,1 % ou moins et N : 0,01 % ou moins, éventuellement au moins un élément choisi dans le groupe constitué de Nb : 0,05 % ou moins, Ti : 0,05 % ou moins, B : 0,0002 % à 0,005 %, Cr : 0,1 % à 0,3 %, et Sb : 0,003 % à 0,03 %, le reste étant constitué de Fe et d'impuretés inévitables ; et
une couche revêtue d'un alliage à base de Zn-Al-Mg formée sur au moins une surface de la tôle d'acier de base à un poids de revêtement par surface de 30 g/m² à 180 g/m², ayant une composition chimique contenant, en % en masse , Al : 3 % à 10 % et Mg : 0,2 % à 0,8 %, et contenant éventuellement au moins un élément choisi dans le groupe constitué de Ca, Sr, Mn, V, Cr, Mo, Ti, Ni, Co, Sb, Zr et B en une quantité totale de 1 % en masse ou moins, le reste étant constitué de Zn et d'impuretés inévitables, et ayant une température de liquidus dans une atmosphère d'air de 400 °C ou moins, et
puis la soumission de la tôle d'acier revêtue à un formage par presse à chaud pour produire l'élément pressé à chaud selon la revendication 1,
dans lequel le poids de revêtement par surface de la couche revêtue d'un alliage à base de Zn-Al-Mg est déterminé conformément à la description.
